

Sept. 6, 1927.

1,641,729

J. E. BRINKER

ORNAMENTED CANDLE AND METHOD OF MAKING SAME

Filed Oct. 27, 1924



INVENTOR  
Jesse E. Brinker,  
By Syngforth Lee, Clinton Miles,  
Attnys.

## UNITED STATES PATENT OFFICE.

JESSE E. BRINKER, OF WHITING, INDIANA, ASSIGNOR TO STANDARD OIL COMPANY,  
OF WHITING, INDIANA, A CORPORATION OF INDIANA.

## ORNAMENTED CANDLE AND METHOD OF MAKING SAME.

Application filed October 27, 1924. Serial No. 746,093.

The present invention relates to improvements in the manufacture of ornamented candles and method of making same and will be fully understood from the following 5 description, illustrated by the accompanying drawing, in which an ornamented candle manufactured in accordance with the present invention is shown.

The present invention is particularly directed to the manufacture of candles having upon their surfaces irregular scale-like incrustations, such candles being described in the patent to Harry F. Blair and Oscar E. Bransky Patent Number 1,520,541, granted December 23, 1924. In that patent, there is described, not only the candle, but also a method of automatically producing the scale-like incrustations on the candle by means of candle dips containing Montan 20 wax.

In accordance with the present invention, it has been found that scale-like incrustations may be produced upon the surfaces of candles, particularly paraffin wax candles, 25 by dipping such candles into molten wax mixtures containing a hydrocarbon wax, such as paraffin wax or petrolatum wax, and from 15 to 50% of carnauba wax. The dip preferably used consists of petrolatum 30 wax (M. P. 120 to 130° F.) and carnauba wax, the latter being present in the proportion of 25%. The proportion of carnauba wax may be varied within the limits above set forth in accordance with the effects 35 which it is desired to produce. In general, it is preferred that the carnauba wax be mixed with petrolatum wax rather than with paraffin wax.

The dip of the above composition is melted, suitable pigments or dyes being incorporated therein, if desired, and a paraffin wax candle of ordinary composition is dipped therein in the usual manner; that is, it is immersed momentarily and withdrawn 45 vertically, the dip forming an external coating on the surface of the candle. As this coating cools the irregular scale-like effect is produced by a breaking-up and marginal curling-up of their regular broken portions 50 of the coating. This is clearly indicated in

the drawing, in which the numeral 5 indicates the candle upon which are the irregular scale-like incrustations 6. Occasionally it is advisable to break off too protruding marginal portions of a candle. If desired, 55 the candle may be subsequently dipped in a molten wax dip of a contrasting color.

## I claim:

1. An ornamented candle having a body consisting largely of paraffin wax and irregular, scale-like surface incrustations of a mixture of hydrocarbon wax and carnauba wax containing 15 to 50% of the latter. 60

2. An ornamented candle having a body portion of paraffin wax and irregular scale-like surface incrustations of a mixture of petrolatum wax and carnauba wax containing 25% of the latter, and a colored coating thereover. 65

3. The method of ornamenting a candle 70 which consists in applying thereto a superficial coating of a molten mixture of a hydrocarbon wax and carnauba wax containing 15 to 50% of the latter, and cooling the candle, said coating thereby forming scale- 75 like incrustations on the candle.

4. The method of ornamenting a candle which consists in applying thereto a superficial coating of a molten mixture of petrolatum wax and carnauba wax containing 15 80 to 50% of the latter, and cooling the candle, said coating thereby forming scale-like incrustations on the candle.

5. The method of ornamenting a candle which consists in applying thereto a superficial coating of molten petrolatum wax and carnauba wax containing 25% of the latter; and cooling the candle, said coating thereby forming scale-like incrustations on the candle. 85

6. The method of ornamenting a candle which consists in applying thereto a superficial coating of molten petrolatum wax and carnauba wax in a mixture containing 25% of the latter, cooling the candle, whereby said coating forms scale-like incrustations on the candle, and subsequently applying a colored coating to the candle. 90 95

JESSE E. BRINKER.